

## UNITED STATES PATENT OFFICE

2,474,538

## ALLOYING MANGANESE WITH MAGNESIUM

Charles H. Mahoney and Gerald L. Lee, Boulder City, Nev., assignors, by mesne assignments, to the United States of America as represented by the Secretary of the Navy

No Drawing. Application June 10, 1944,  
Serial No. 539,786

2 Claims. (Cl. 75—168)

1

This invention relates to magnesium alloys containing manganese, and has for its object the provision of certain improvements in alloying manganese with magnesium.

Manganese is commonly included in most magnesium base alloys employed for structural and other commercial uses. Binary magnesium-manganese alloys commonly contain 1 to 3% manganese, and magnesium base alloys commonly contain from 0.05 to 3% manganese, with, for example, 0.1 to 12% aluminum and 0.05 to 5% zinc. The amount of manganese included in these alloys is limited on the higher side by the solubility of manganese in magnesium and in magnesium base alloys and on the lower side by the amount required to impart the desired corrosion resistance and other properties to the alloy. In general, magnesium alloys contain from 0.05 to 3% manganese, while the magnesium base alloys containing aluminum customarily contain from 0.05 to 1.0% manganese.

The direct alloying of metallic manganese with magnesium is attended by considerable difficulties, and while the literature casually mentions the melting together of metallic manganese and magnesium or the introduction of metallic manganese to molten magnesium or alloys thereof, the customary industrial practice is to introduce the manganese in the form of a reducible manganese compound, commonly manganous chloride. Thus, dehydrated manganous chloride, in flake or granular form, is placed on the surface of the molten magnesium, or magnesium alloy, the magnesium replacing manganese in the manganous chloride with the liberation of metallic manganese which is then available for alloying with the magnesium. The resulting magnesium chloride is heavier than the molten metal and sinks to the bottom of the bath. Manganous chloride crystallizes with four molecules of water ( $MnCl_2 \cdot 4H_2O$ ), and while part of the water of crystallization is easily driven off, complete dehydration is difficult without converting some of the chloride to oxide. Moreover, the flake or granular dehydrated manganous chloride is of light weight and dusts easily thereby contaminating other melts in the plant in which manganese is not desired, or is objectionable. The replacement of manganese by magnesium is never complete, and with good alloying practice efficiencies of about 70% can be accomplished. As a consequence, the use of manganous chloride is expensive, and the results obtained leave much to be desired with respect to accurate control of the alloy composition.

2

Where attempts have been made to alloy metallic manganese directly with magnesium or its alloys, much of the manganese is oxidized. Moreover, because of its relatively high specific gravity, much of the manganese settles rapidly through the molten magnesium and collects in the sludge or flux layer at the bottom where it tends to become coated with the chloride fluxes. As a result, low and unpredictable efficiencies are attained, and accurate control of the alloy composition is impossible. In an attempt to overcome these difficulties, manganese has been introduced into the molten magnesium in the form of an intermediate alloy with another metal as a hardener. However, the use of the intermediate manganese alloy is limited to alloys in which the presence of the other hardening metal is contemplated, and moreover the additional cost of producing the intermediate alloy is objectionable.

The present invention aims to provide a commercially satisfactory and economical method of directly alloying metallic manganese, and particularly electrolytically produced manganese, with magnesium. As a result of our investigations, we have discovered that the presence of aluminum in molten magnesium adversely affects the direct alloying of manganese with the magnesium by lowering or retarding the solubility of the manganese. We have further found that metallic manganese in a moderately coarse condition can be directly alloyed with magnesium with satisfactory efficiency. For optimum results, the molten magnesium should be substantially free of chloride-containing fluxes, and the temperature of the molten magnesium should be above 740° C. before adding the metallic manganese.

Based on the foregoing discoveries, the present invention involves directly alloying metallic manganese with magnesium by adding relatively coarse manganese to molten magnesium at a temperature of from 750 to 800° C. and prior to adding aluminum. The magnesium should be essentially aluminum-free for optimum alloying efficiency, although reasonably satisfactory results can be obtained with magnesium containing only a few tenths of a percent of aluminum. The metallic manganese, preferably electrolytic manganese, is crushed to moderate fineness, so that approximately all passes through a 4 mesh standard Tyler screen or sieve and a minimum passes a 150 mesh screen. We have found that too finely ground manganese, that is through or minus 150 mesh, oxidizes rapidly with result-

ing low alloying efficiency. On the other hand, too coarse particles, that is on or plus 4 mesh, sink too rapidly through the molten metal for good alloying efficiency. Accordingly, we have determined that substantially all of the metallic manganese should be minus 4 mesh and plus 150 mesh for optimum alloying efficiency.

In practicing the invention the magnesium metal is melted under a suitable protective cover (inert gas or flux). The molten metal is then heated to a temperature of between 750° C. and 800° C., and the calculated amount of moderately coarse metallic manganese (preferably electrolytic manganese) is added. It is necessary prior to adding the manganese that the magnesium metal be refined as free of chloride-containing fluxes as possible in order to achieve maximum manganese efficiency. The manganese is preferably laid on the bare surface of the clear molten magnesium, and gradually sinks therethrough. Preferably, to minimize burning losses, a suitable protective cover of inert gas or flux is applied to the surface of the molten metal as soon as the manganese is added. After an interval of 5 to 10 minutes, the molten alloy is agitated by stirring or plunging. The agitation may be done by plunging with a hand tool or by mechanical stirring. If aluminum, zinc or other metal additions are to be made to the alloy, they are added to the molten magnesium-manganese alloy if maximum manganese efficiency is to be obtained.

Although a substantially chloride-free molten magnesium metal is necessary in order to achieve maximum alloying efficiency, alloying efficiencies of 70% or better can be obtained by adding to the molten magnesium metal a mixture of relatively coarse manganese and commercial magnesium refining flux, the proportion of manganese exceeding 50% of the mixture. We have found that the customary thin chloride melting flux tends to set the manganese and thus impairs the alloying effort. Hence, in the preferred practice of the invention, we carefully refine out any chloride melting flux in order to obtain maximum alloying efficiencies. On the other hand, we have found that the customary thick refining fluxes do not greatly impair the alloying efficiency of the manganese. These commercial refining fluxes consist generally of a chloride salt base, for example a mixture of alkali chlorides and alkali-earth chlorides, and contain 20 to 40% of inspissating agents such as magnesia and calcium fluoride (e. g. fluorite). When such a mixture of relatively coarse manganese and commercial refining flux is added to the molten magnesium metal, the flux apparently protects the manganese fines, such as pass a 150 mesh sieve, from oxidation or loss, and the presence of certain amounts of such fines does not deleteriously affect the efficiency of the alloying effort and may be tolerated. The mixture of moderately coarse metallic manganese, preferably electrolytic manganese, with commercial magnesium refining flux constitutes a new and useful article of commerce for the direct introduction of manganese into molten magnesium metal in accordance with the principles of the invention.

As a specific example of the practice of the invention in the manufacture of a binary magnesium-manganese alloy containing approximately 1.5% manganese, 150 pounds of electrolytic magnesium metal essentially aluminum-free was melted under a chloride-containing magnesium melting flux, and the resulting melt was heated

to a temperature of approximately 760° C. At this temperature, the magnesium melt was refined by stirring in a magnesium refining flux containing magnesium oxide and calcium fluoride along with chloride-containing base salts. To this refined magnesium melt was then added 3 pounds of electrolytic manganese crushed to pass a 30 mesh sieve and essentially all coarser than 100 mesh. In this example, the metal was immediately stirred by hand plunging for a few minutes and re-stirred at 10 minute intervals for approximately 30 minutes. At the end of 30 minutes a sample of the metal showed 1.4% manganese, and 20 minutes later, after intermittent stirring, the metal contained 1.68% manganese. The metal was then superheated at a temperature of 900° C., cooled to 740° C., and cast. The cast metal contained 1.68% manganese, the manganese alloying efficiency being thus about 86%.  
20 As another example, 150 pounds of essentially aluminum-free electrolytic magnesium metal was melted and heated to a temperature of 780° C., using a chloride-containing magnesium melting flux for protection against oxidation. The metal was refined, using a commercial magnesium refining flux containing magnesium oxide, calcium fluoride in addition to the chloride-containing base salts. To this magnesium melt was added sufficient electrolytic manganese crushed to pass a 12 mesh sieve to give theoretically 0.3% manganese in the finished alloy. In this example, the melt was immediately stirred by hand plunging, and after intermittent stirring for 15 minutes, pure ingot aluminum and pure ingot  
25 zinc were added to give an alloy containing approximately 4% aluminum and 0.5% zinc. After alloying the aluminum and zinc, a sample of the metal showed the alloy to contain 0.25% manganese. The metal was then heated to 815° C., cooled to 720° C., and cast. The resulting product contained 0.25% manganese, the manganese alloying efficiency being thus approximately 83%.

In another example, 150 pounds of essentially aluminum-free electrolytic magnesium metal was melted and heated to 760° C., using a commercial magnesium melting flux for the purpose. The molten metal was refined, using a commercial magnesium refining flux. Sufficient electrolytic manganese, crushed to pass a 12 mesh sieve, to give theoretically 2.0% manganese in the alloy was then mixed with approximately 1 pound of the commercial magnesium refining flux and the mixture was stirred into the molten metal. The metal was stirred at 5 minute intervals and after 25 minutes a sample of the metal showed a manganese content of 1.25%. The metal was stirred again and, after 20 more minutes, a sample of the metal showed 1.6% manganese. The metal was then heated to 900°, cooled to 720° C. and cast into ingots. The manganese content of the ingots was 1.6%, the manganese alloying efficiency being approximately 80%.

The invention provides an improved method of alloying manganese with magnesium in a rapid, effective and economical manner. It is particularly characterized by the high and superior manganese alloying efficiency, that is the ratio of the amount of manganese actually present in the finished alloy to the amount of metallic manganese initially added to the molten magnesium. Moreover, the invention enables the production of magnesium-manganese and magnesium base alloys containing definite amounts of manganese with high alloying efficiencies. No dust is raised

in the necessary handling of the moderately coarse metallic manganese, and hence other melts in the plant are not contaminated with manganese. The manganese alloys promptly with the magnesium, alloying times of from 15 to 45 minutes being usually adequate, depending to some extent upon the percentage of manganese to be included in the alloy. With manganese contents up to about 1%, it is preferable to place the manganese upon the bare surface of the clean molten magnesium, immediately apply a protective cover, and wait for 5 to 10 minutes before stirring or agitating. Alloying is completed in about 15 minutes. With higher manganese contents, earlier and more frequent stirring and longer alloying times are usually desirable.

We claim:

1. The improvement in permanently alloying manganese with magnesium which comprises introducing crushed metallic manganese into essentially aluminum-free molten magnesium at a temperature of from 750 to 800° C., the particle size of the manganese being in the range minus 4 mesh and plus 150 mesh.
2. The improvement in alloying manganese with magnesium which comprises adding crushed metallic manganese of a particle size which is in the range of minus 4 mesh and plus 150 mesh to molten magnesium and stirring the melt to facilitate alloying.

CHARLES H. MAHONEY.  
GERALD L. LEE.

## REFERENCES CITED

The following references are of record in the file of this patent:

## UNITED STATES PATENTS

| Number    | Name                  | Date          |
|-----------|-----------------------|---------------|
| 2,029,898 | Schmidt et al. -----  | Feb. 4, 1936  |
| 2,235,508 | Zeppelin et al. ----- | Mar. 18, 1941 |
| 2,236,831 | Nelson -----          | April 1, 1941 |
| 2,262,106 | Leech -----           | Nov. 11, 1941 |
| 2,267,862 | Hanawalt et al. ----- | Dec. 30, 1941 |
| 2,317,980 | Dean et al. -----     | May 4, 1943   |
| 2,370,320 | Moss -----            | Feb. 27, 1945 |
| 2,373,515 | Stroup et al. -----   | Apr. 10, 1945 |

## FOREIGN PATENTS

| Number  | Country             | Date          |
|---------|---------------------|---------------|
| 336,498 | Great Britain ----- | Oct. 16, 1930 |

## OTHER REFERENCES

- 20 "Technology of Magnesium and its Alloys," 1940, pages 313-319 inclusive, 321 and 322; a translation by F. A. Hughes & Co., Published London, England, of the German compilation of Beck: "Magnesium und Seine Legierungen."
- 25 Dasher: "Directions for Laboratory Mineral Sizing," U. S. Bureau of Mines Circular No. I. C. 7224, Nov. 1942, 16 pages (pages 5 and 6 relied upon).
- 30